

# UNITED STATES PATENT OFFICE.

HARRY P. CORLISS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,228,183.

Specification of Letters Patent.

Patented May 29, 1917.

No Drawing.

Application filed March 21, 1917. Serial No. 156,491.

*To all whom it may concern:*

Be it known that I, HARRY P. CORLISS, a citizen of the United States, residing in Pittsburgh, county of Allegheny, and State 5 of Pennsylvania, have invented certain new and useful Improvements in the Flotation of Minerals; and I do hereby declare the following to be a full, clear, and exact description of the invention, such as will enable 10 others skilled in the art to which it appertains to make and use the same.

This invention relates to the concentration of minerals, such as sulfid ores and the like, by flotation and is based upon the discovery that improved results can be obtained by carrying out the flotation operation with the addition to the ore or mineral pulp of alpha-naphthylamin either alone, or with added amounts of "oil". The alpha-naphthylamin is a non-oleaginous solid material which can nevertheless be distributed throughout the ore pulp with such uniformity that minimum amounts are required for effecting the concentration of the mineral by flotation. It is not necessary that chemically pure naphthylamin be used, but the commercial product (made, for example, by reducing nitro-naphthalene) can be used in its crude or unrefined state, the reduction being effected for example by means of iron and hydrochloric acid. The product thus produced is found to be substantially as efficient as a product of higher purity.

In using the alpha-naphthylamin it may be added to the ore, either alone or with added amounts of oil, in any suitable manner, so that it will be thoroughly and uniformly distributed throughout the ore pulp. The mixture is then subjected to a flotation 35 operation as in an ordinary Calow cell or in apparatus where the air is incorporated in the ore pulp by mechanical agitation. With some ore pulps it may be desirable to add either small amounts of acids or of alkalis, depending upon the nature of the ore pulp to be treated.

The amount of alpha-naphthylamin used may vary somewhat, for example, between

one-half pound and one and one-half pounds per ton of ore (that is, calculated on the 50 weight of the ore and not of the ore pulp).

The results obtained by carrying on the flotation with the addition of alpha-naphthylamin or with alpha-naphthylamin and added oil, indicate that higher grades of 55 concentrates and better recoveries can be obtained than with the usual oil mixtures and even with most, if not all, of the best oil mixtures.

It is a further characteristic of the invention that the froth obtained is readily broken up and the alpha-naphthylamin recovered therefrom, so that it is available for use in the treatment of further amounts of ore. That is to say, the circuit water recovered from the concentrate and even that recovered from the tailings contains notable amounts of alpha-naphthylamin which can thus be returned to the process with resulting economy in the amount required to be 70 added for subsequent operations.

In applying the alpha-naphthylamin it may be introduced into the tube mill in which the ore is being ground or it may be otherwise introduced into the ore pulp 75 in any suitable way, as, for instance, by first digesting it in hot water and mixing the product with the ore pulp just before it enters the flotation cell.

Having thus described my invention, what 80 I claim is:

1. The method of effecting the concentration of minerals by flotation, which comprises adding to the mineral pulp a small amount of alpha-naphthylamin and subjecting 85 the resulting mixture to a flotation operation; substantially as described.

2. The method of effecting the concentration of minerals by flotation, which comprises adding to the mineral pulp a small 90 amount of alpha-naphthylamin and of oil and subjecting the resulting mixture to a flotation operation; substantially as described.

In testimony whereof I affix my signature. 95  
HARRY P. CORLISS.